

Nov. 10, 1959

M. YEZEK ET AL

2,912,347

PROCESS OF PRODUCING GLOSSY WAX-COATED PAPER

Filed June 3, 1957



INVENTORS

MILTON YEZEK  
WALTER C. UTSCHIG

BY *Frederick F. Mack and*  
*Michael J. Quilligan* ATTORNEYS

1

2,912,347

## PROCESS OF PRODUCING GLOSSY WAX-COATED PAPER

Milton Yezek and Walter C. Utschig, Battle Creek, Mich., assignors to General Foods Corporation, White Plains, N.Y., a corporation of Delaware

Application June 3, 1957, Serial No. 663,269

8 Claims. (Cl. 117—64)

The present invention relates to the production of glossy wax-coated paper.

In making wax-coated papers for use as a wrapping material for commodities it is highly desirable that the wax-coating offer a high degree of gloss and yet be free of any imperfections which detract from the appearance and utility of the wax-coated paper. Heretofore it has been proposed to provide glossy wax-coated paper by chilling a paper web, once the hot wax composition has been applied thereto, by passing the coated web through a cold water bath or over chilling rolls. But these procedures suffer from a number of disadvantages. In the case of cold water cooling, gloss is attainable with some coating formulas but "crow's feet" are evident on the waxed surface, and at high production rates the population of crow's feet is high. With conventional cold roll cooling high glosses are not attainable. Another possible procedure is "cast-coating;" in "cast-coating," a molten wax coating previously applied to the paper web is solidified while in contact with the surface of a smooth, polished casting surface and, after the coating has set, the wax-coated paper is peeled from the casting surface. However, in cast-coating there is a likelihood, due to poor synchronization between various roll speeds and the web, that the web of paper will move relative to the surface of the cold roll; as the wax composition solidifies and crystallizes there will be a severe reduction in the smoothness or regularity of the surface of the coating and the gloss will be considerably reduced, if not destroyed; this is particularly the case at high production rates. When employing a cast-coating procedure it is also required that the roll be operated at a slow enough speed to allow the wax composition to solidify; otherwise "picking," virtual peeling of portions of the wax composition from the coating onto the roll, will occur as the wax-coated web itself is peeled from the roll. This accumulation of coating composition impairs the efficacy of the casting surface on subsequent revolutions of the casting roll.

These problems probably stem from a number of factors. The bond between the wax composition and the paper web, the release properties of the wax composition or the casting surface or both, and the tensile strength of the wax composition itself more or less influence the degree of gloss obtainable at a given rate of web travel.

Because of the discontinuity of the coating resulting from cast-coating at high production speeds, there is a decrease in the water vapor transmission resistance of the wax-coated paper. It is desirable, therefore, to provide a wax coating process where, in addition to improved gloss and over-all appearance of the wax-coated paper, there is no accompanying decrease in its water vapor transmission resistance.

It has now been discovered that a smooth, extremely glossy wax-coated paper can be produced at high rates of speed by applying a hot melt wax coating composition onto a web of paper and "shock-cooling" the coating composition while it is being cast on a portion of an endless coating member. This shock-cooling is achieved by first

2

urging the coated paper web with the coating composition in a molten state into immovable relation with the endless casting member, the latter having a smooth mirror-finished surface which contacts the coating composition. 5 Such urging is preferably effected by means of the pressure of an impression roll. The coating member is maintained on its smooth surface at temperatures below the point of crystallization of the wax coating composition. The web of coated paper and the smooth surface of the casting member are immediately thereafter further cooled by water also maintained at temperatures substantially below the point of crystallization of the coating composition, the water being caused to contact the web of paper from the side thereof further removed from the smooth surface of the casting member and after contact by the wax coating composition with the smooth casting surface. By virtue of the shock-cooling of the coating which takes place, the web and the coating composition are maintained in immovable contact with the smooth surface of 10 the casting member until a temperature substantially below the heat of fusion of the coating composition is reached and the coating composition is crystallized, whereby a slight bond is created between the coating and the contacting surface of the paper web, and the coating itself has developed sufficient tensile strength to overcome this bond without any adverse effects when the wax-coated paper is later peeled from the casting surface. The cooled wax-coated web of paper is eventually peeled from the casting member, preferably after the web leaves 15 the zone of application of the cold water, the coated paper being preferably peeled under uniform tension from the casting member under the influence of a pressure roll maintained against the web of wax-coated paper.

Thus, the coating composition, e.g., a wax composition 35 of paraffin-blended with additives such as microcrystalline wax and/or polymeric compositions such as polyethylene, is essentially cooled quite rapidly after contact with the smooth surface of the casting member from both sides of the film of coating composition and the latter is maintained relatively immovable during crystallization between a substantial portion of the casting member and the web of paper. As a result of this process it is found that a surface is produced on the coating which is extremely glossy, smooth and continuous, and the glossy surface is entirely free of crow's feet. The process is characterized 40 by improved release properties between the smooth surface of the casting member which is preferably a cold roll having a smooth mirror-finished surface thereon. In lieu of a roll, an endless belt also having a smooth mirror-finished surface may be employed. The continuity of the eventual coating is such that it offers superior resistance to water vapor transmission despite the finding that the wax-coated paper is capable of being produced at high rates.

It appears that by shock-cooling the molten wax coating composition it is caused to go through, or give up, its heat of fusion and crystallize rapidly thereby offering unusually glossy surfaces. Shock-cooling also serves to rapidly solidify the coating intermediate the paper web and the casting surface and thereby creates a bond which reduces any tendency toward relative movement reducing or destroying gloss. Consequently, high rates of web travel in processing can be employed and at such rates high gloss results. Advantageously, it has been found that, as the rate of web travel is increased, gloss is correspondingly increased when the wax-coated paper is shock-cooled. Furthermore, by reason of the rapid cooling offered at high rates of web travel the wax coating quickly develops adequate tensile strength to resist picking of the composition onto the casting member and any premature distortion of the coating composition due to improper synchronization between the rolls and the paper web.

The invention will be more clearly understood by reference to the drawing which is a schematic illustration of a preferred coating assembly which can be employed to produce the improved wax-coated paper of the present invention.

The coating assembly comprises a pair of waxing nip rolls 1 which are employed to distribute a molten wax composition on both sides of a web of paper passing between the waxing rolls. The molten wax composition can then be passed under a heated steel polishing roll 2 which further distributes the wax composition over the surface of the web of paper. The web of paper then travels over an impression roll 3 which can be a rubber roll and around a large segment of the surface of a large diameter cold roll 4, the web of paper then being peeled from the surface of the cold roll 4 under the control of a soft rubber wringer roll 5. The cold roll 4 is chilled by a brine circulating within the roll, the temperature to which the roll is cooled being anywhere from between -30° F. to +32° F. and being generally below the fusion point of the wax composition. The cold roll 4 and the web of wax-coated paper trained therearound are submerged in a cold water bath 6 also maintained at a temperature below the fusion point of the wax composition. In this connection, ordinary cold water just above 32° F. is preferably employed, although a cold brine solution may also be employed to advantage in the water bath.

The wax coating composition employed in accordance with the present invention may be molten paraffin wax or paraffin wax having certain additives blended therewith such as microcrystalline wax or synthetic resins such as low molecular weight polyethylene. In general the gloss of all wax coating compositions is significantly increased when the web of wax coated paper is shock-cooled by being submerged in the cold water bath 6 while being maintained in intimate contact with the cold roll 4. The cold roll 4, serving as the casting member on which is provided the smooth surface necessary to produce the high gloss of the present invention, preferably has incorporated around its periphery a continuous and extremely smooth sheet of material such as vinyl acetate. This sheet should possess good release properties and offer a degree of smoothness which will result in a continuous surface on the film of coating which is cast onto the web of paper while it is maintained in immovable relationship to the cold roll 4. Instead of a sheet of vinyl acetate, other compositions capable of offering a smooth, mirror-finished surface and good release properties such as a sheet of copper or aluminum foil may be employed as well as a lacquer of silicone grease or other resin, or less preferably a polished metal roll or a nickel or chromium plated roll. In general the casting surface of the cold roll 4 should have a mirror-like finish and should have a surface which when cooled to substantially below the fusion point of the coating composition adheres to the coating with only a slight bond such that the wax-coated paper can be readily peeled from the cold roll 4. As a consequence, although the web of paper with its coating is submerged in a bath of cold water for shock-cooling, sufficient bond exists between the coating and the roll to prevent the entry of excess moisture therebetween, thereby avoiding any dull spots or areas on the surface of the coating. This bond also acts to avoid any relative movement between the endless casting member and the web of paper due to poor synchronization between the casting member and the paper web.

In order to assure absence of relative movement between the web of paper, the coating and the cold roll 4, it is preferred that the latter be positively driven and that the rubber impression roll 3 and the wringer roll 5 be driven idly by contact with the cold roll 4 through inter-mediation of the web of paper and the coating. The rubber impression roll 3 is preferably maintained at a temperature generally above the melting point of the wax composition so as to assure that the surface of the coating

is complementary to the surface of the cold roll 4. Accordingly, rubber pressure roll 3 is maintained just above the surface of the cold water bath so as to avoid premature solidification of the molten wax composition before it has had an opportunity to conform to the smooth surface of the casting member or cold roll 4. In order to insure an adequate degree of conformity of the coating composition to the surface of the cold roll, positive pressure is applied to the rubber roll 3.

Pressure is also applied to the rubber wringer roll 5 and this roll is also located above the surface of the cold water bath so as to avoid the collection of moisture on the casting surface of the cold roll 4 after the wax-coated paper is peeled therefrom. It is most desirable that steps be taken to avoid accumulation of any moisture on the casting surface of the cold roll 4. Moreover, the axis of wringer roll 5 should be substantially parallel to the axis of the cold roll 4 so that the web of wax-coated paper is peeled without any eccentricity from the cold roll, thereby avoiding any distortion of the surface of the wax coating and tearing of the web.

Although the shock-cooling which takes place while the web of paper and its wax coating is cast on the surface of cold roll 4 is quite considerable, it will still be desirable to employ a series of conventional chilling rolls 7 and doctor blades 8 so as to assure that the coating composition is cooled to the degree that it will not "block" or retain tackiness after the wax-coated paper is put on a winding roll. Thus, the large diameter chilling roll in combination with the cold water bath crystallizes the wax by taking it rapidly through its heat of fusion and cools the wax substantially therebelow to remove any sensible heat and thereby assures that the heat of fusion is removed. Thereafter the series of chill rolls 7 serve to further cool the coating so that it will not block and the gloss achieved will be preserved by avoiding any tendency of the wax coating to migrate after the wax-coated paper is wound onto a roll.

In the preferred modification of the present invention a molten wax composition comprising about 50 parts by weight of paraffin (M.P. 140°-145° F.) and 50 parts by weight of microcrystalline wax (M.P. 145°-147° F.) is applied to a web of paper or paperboard which may range from 15 to 300 lbs. per 3000 sq. ft. Preferably a minor proportion of polyethylene ranging in average molecular weight from 2000 to 21,000 is also employed, it being found that the polyethylene serves to promote some degree of resistance to blocking as well as additional gloss to the coating. The eventual wax-coated paper has a thickness ranging anywhere from 0.001 to 0.025 inch. When employing the aforementioned preferred wax composition the rubber impression roll 3 is preferably heated to a temperature between 150°-250° F. to assure that the wax composition is sufficiently molten and plastic in nature to assume the smoothness of the surface of the cold roll 4. The rubber impression and wringer rolls preferably have a diameter ranging from 4 to 10 inches and the cold roll 4 has a diameter ranging from about 1½ to 6 feet, the cold roll being immersed in a bath of cold water and surrounded by the web of paper on the majority of its circumference during its operation. The cold water bath may have added thereto organic materials like ethylene glycol which allow the cold water to be maintained sufficiently cool and yet avoid freezing of the coolant. The cold roll 4 can be chilled with a suitable refrigerant such as a brine which acts to maintain the temperature well below the point of crystallization of the wax composition.

The pressure roll 3 is urged with the pressure of 50 to 200 lbs. per linear inch against the cold roll 4 and preferably has a hardness in the order of 60 to 100 (Shore A durometer hardness) in order to assure that the wax coating composition is applied uniformly and in a continuous film against the smooth surface of the cooling roll 4, care being exercised to avoid crystallization of

the wax composition before it assumes a smoothness like that of the cold roll on which it is to be cast. Thereafter the wax composition is rapidly chilled by the cooling bath and the cold roll absorbing its heat so that the wax quickly goes through a plastic condition to assume a crystalline state having very small crystals. By virtue of the dual cooling mediums, the heat absorbed on the casting surface of the cold roll 4 is quickly transferred to the coolant circulated within the roll and to the cold bath. During the shock-cooling process the wax-coating composition sets at such a high rate that opportunity for any relative movement between the web of paper, the coating or the casting surface of the cold roll is nil, such that during crystallization of the wax composition little, if any, displacement thereof occurs. The coating sets with a slight bond against the smooth casting surface and can be readily peeled therefrom by training the wax-coated paper around the wringer roll 5 from the cold roll. When the aforementioned preferred wax composition is used it is possible to operate the cold roll at extremely high rates of speed and produce very glossy wax-coated paper at a rate in the order of 1000 linear feet per minute and above.

Thereafter, the web of glossy wax-coated paper is cooled, when the preferred wax composition is used, to a temperature in the order of 115° F. and below, the doctor blade 8 being employed to remove any moisture condensing or otherwise collected on the surface of the wax-coated paper.

Although various formulations for wax coating compositions can be employed in the present invention to produce improved results with respect to the degree of gloss obtained, and although these compositions usually contain paraffin as a principal constituent, it is preferred to employ microcrystalline wax in the formulation in combination with the paraffin. The preferred microcrystalline wax is one which has been de-oiled since this type of wax results in a coating of relatively high tensile strength. In general blends of paraffin and microcrystalline wax result in higher gloss and allow higher production rates in the present process than in instances where paraffin wax is employed solely.

It will be understood that the term "paper web," or "web of paper," as used herein, includes both continuous and discontinuous webs, as the advantages of the invention are obtainable with either.

While the present invention has been described with particular reference to specific examples, it is not to be limited thereby, but reference is to be had to the appended claims for a definition of its scope.

What is claimed is:

1. The method of producing a glossy wax-coated paper which comprises applying a hot melt wax-coating composition onto a web of paper, bringing the resulting coated surface of the paper web with positive pressure and with said composition in a molten state into intimate contact with a rapidly moving endless casting member having a smooth mirror-finished surface, the molten wax composition being thereby uniformly distributed between the web and the surface of the casting member and being solidified rapidly by cooling said casting member on its smooth surface to a temperature below the point of crystallization of the wax-coating composition at least after contact therewith and by simultaneously cooling the uncoated surface of said web during said contact by the application thereto of water maintained at a temperature substantially below the temperature of crystalli-

zation of said coating composition, moving said web and said casting member at the same linear speeds with said composition solidifying between them in contact with said smooth surface whereby said web and said coating composition are maintained in intimate immovable relation with said smooth surface and entry of cooling water between them is prevented until the heat of fusion of said coating composition is removed and it is crystallized, and thereafter peeling the cooled coated web of paper from said casting member.

2. The method of claim 1 wherein the wax-coating composition comprises paraffin.

3. The method of claim 1 wherein the wax-coating composition comprises a blend of paraffin and microcrystalline wax.

4. The method of claim 1 wherein said positive pressure is provided and said coating composition is distributed by an impression roll urging said coated web into initial contact with said casting member.

5. The method of producing a glossy wax-coated paper which comprises applying a hot melt wax-coating composition onto a web of paper, bringing the resulting coated side of the paper web, with said composition in a molten state, into intimate immovable relation with a segment of the surface of a rapidly rotating mirror-finished smooth roll so that said coated side makes contact with the roll surface, said coated paper web being urged into contact with said roll under positive pressure from an impression roll acting to uniformly distribute the wax-coating composition between the web and the surface of the mirror-finished roll, said mirror-finished roll being maintained on its smooth surface at a temperature substantially below the point of crystallization of the wax coating composition, thereby to cool said coated paper web, said web of coated paper and said smooth surface then being simultaneously and further cooled by moving the same through a body of cold water maintained at a temperature substantially below the temperature of crystallization of said coating composition, said body of cold water making contact with said web of paper on the side thereof further removed from said smooth surface, said web and said coating composition thereon being maintained in immovable contact with, and relatively to, said smooth surface and being submerged in said body of cold water until the heat of fusion of said coating composition is removed and it is crystallized, and thereafter peeling the cooled coated web of paper from said mirror-finished roll after said web leaves the zone of application of said water.

6. The method of claim 5 wherein the crystallized wax-coated paper web is peeled under tension from the mirror-finished roll by causing said web to travel over an idling pressure roll whose axis is parallel to the axis of the mirror-finished roll and which is resiliently maintained thereagainst.

7. The method of claim 6 wherein the wax-coating composition comprises paraffin.

8. The method of claim 6 wherein the wax-coating composition comprises paraffin and microcrystalline wax.

#### References Cited in the file of this patent

#### UNITED STATES PATENTS

|           |              |               |
|-----------|--------------|---------------|
| 2,642,366 | Rumberger    | June 16, 1953 |
| 2,753,275 | Wiles et al. | July 3, 1956  |
| 2,829,980 | Redd         | Apr. 8, 1958  |

UNITED STATES PATENT OFFICE  
CERTIFICATE OF CORRECTION

Patent No. 2,912,347

November 10, 1959

Milton Yezek et al.

It is hereby certified that error appears in the printed specification of the above numbered patent requiring correction and that the said Letters Patent should read as corrected below.

Column 1, line 72, and column 2, line 6, for "coating", each occurrence, read -- casting --; column 2, line 57, for "head" read -- heat --; column 3, line 43, for "wil" read -- will --; line 69, for "later" read -- latter --; column 6, lines 30 and 31, for "mirro-finished" read -- mirror-finished --.

Signed and sealed this 3rd day of May 1960.

(SEAL)

Attest:

KARL H. AXLINE  
Attesting Officer

ROBERT C. WATSON  
Commissioner of Patents